

# UNITED STATES PATENT OFFICE.

OSWALD SILBERRAD, OF BUCKHURST HILL, ENGLAND.

## PROPELLANT EXPLOSIVE.

Specification of Letters Patent. Patented Aug. 17, 1920.

1,349,983.

No Drawing.

Application filed September 10, 1919. Serial No. 322,947.

To all whom it may concern:

Be it known that I, OSWALD SILBERRAD, consulting chemist, a subject of the King of England, and residing at Buckhurst Hill, 5 in the county of Essex, England, have invented certain new and useful Improvements in Propellant Explosives, of which the following is a specification.

My invention relates to explosives of the 10 propellant class and has for its object the production of propellants which give no flame and little smoke when fired in guns or howitzers of a suitable caliber and design, or rifles or shot guns.

15 In particular my invention relates to the production of a "flameless powder" of such properties that when made of the required size the correct charge will when fired in a suitable weapon give the present service 20 velocities without flame and at the same time produce little if any more smoke than is produced by the so called smokeless powders at present in use. By the term "suitable weapon" I include any rifle or shot gun 25 at present in use, any howitzer at present in use up to and including 6", and/or any gun at present in use up to and including the 3.3". A "flameless powder" is not flameless if burned in the open, nor is it flameless 30 if fired in guns where the cooling effect due to the energy absorbed by the shot is insufficient to reduce below their ignition point the temperature of the gases evolved upon the firing of said propellant in said guns. It 35 will be observed therefore that a "flameless powder" as herein defined is not necessarily flameless if fired in guns of larger caliber than those specified in above definition or at pressures higher than the normal working 40 pressures. And throughout this application I use the term "flameless powder" to denote a propellant which will give the aforesaid results whether said powder be flameless in guns and/or howitzers of larger caliber 45 or not, and include propellants which give the aforesaid results either alone or with the admixture of any given proportion of any given propellant which when fired alone produces flame.

50 Heretofore all attempts to obtain this effect have been based on the use of salts of metals such as the carbonate or bicarbonate of sodium or potassium or resinate of sodium or calcium: By this means powders 55 have been produced which are flameless in

some of the smaller guns. Such powders are, however, of very little use owing to the enormous amount of smoke simultaneously produced.

I have discovered how to produce a flameless powder without the introduction of any metallic salts or any compound which leaves a relatively non-volatile residue; in short, the flameless propellant which I produce bears a similar relationship to the known 65 flameless powders as the present smokeless powders bear to the old black powder.

My invention therefore relates to the production of a new article of warfare and commerce, namely, a "flameless powder" as 70 hereinbefore defined.

As a result of a very exhaustive study of the interdependent equilibria which control the composition of the products of the auto-combustion of propellants under the conditions pertaining in artillery practice, I have discovered that the aforesaid result can be arrived at by suitably raising the ratio of

$\text{H}-\overset{\text{I}}{\underset{\text{|}}{\text{C}}}-\text{OH}$  groups to  $\text{N}=\overset{\text{O}}{\text{C}}$  groups, and

further that this may conveniently be achieved by introducing a sufficient quantity of one or more suitable compounds into any of the existing so called smokeless powders and/or propellants. By the qualification "suitable" above I mean otherwise suitable—i. e. solid or soluble in the gelatinizing 90 agent and sufficiently non-volatile and non-hygroscopic to be used reasonably in a propellant powder. It is only such bodies hav-

ing also a preponderance of  $\text{H}-\overset{\text{I}}{\underset{\text{|}}{\text{C}}}-\text{OH}$

groups as are intended to be included herein, such compounds are starch, mannite, sugar, glucose, cellulose, lignocellulose, cellulose 100 acetate and the like. From the above data it will be simple to select other suitable compounds though of the aforesaid I find that starch is the most suitable and produces a powder which as well as being possessed of 105 the best keeping properties also gives rise to less smoke than any other "flameless powder" I have been able to produce and far less than anything heretofore produced; I 110 therefore prefer to use starch,

Further, I have discovered that in order to render the flameless powder as smokeless as possible it is necessary to incorporate the starch or the like into the powder and that if said starch or the like be merely added to the finished propellant the interaction of the said starch or the like on autocombustion is not complete and much carbonaceous matter separates as smoke on firing. On the other hand I find that quite satisfactory results can be obtained by incorporating an excess, say for example, twice the quantity required of said starch or the like with any given propellant mixture and then making up charges or cartridges of a mixture of this product together with any ordinary propellant or smokeless powder in the desired proportions, namely in the above example in equal proportions, each propellant being of the desired size. From this it will be observed that it is not necessary for the starch or the like to be evenly distributed throughout the entire charge, but that the charge may be made up of a mixture of a propellant containing an excess of starch or the like with one containing a deficiency or none at all, as for example any of the smokeless powders at present in use providing always that the quantity of starch or the like in the entire charge be such that the temperature of the gases emitted from the muzzle is below their ignition point as hereinbefore set forth.

In carrying my invention into effect, therefore, I prefer to use starch and to incorporate said starch with any suitable propellant material or mixture which without such addition would produce a propellant such that if fired in the aforesaid weapons would produce flame.

I have found that the quantity of starch or the like to be added depends on the pyrometric value of the original propellant, material or mixture used and must be sufficient to reduce the temperature of the gases emitted from any given gun to below the ignition point of said gases when the resultant product will be found to be a "flameless powder" as hereinbefore defined. The quantity can therefore be calculated by those familiar with thermodynamics and internal ballistics; thus, using Mallard and Le Chatelier's figures for the specific heat of gases, we find that the pyrometric value of M. D. cordite under conditions similar to those pertaining in artillery practice is approximately 2300° C., hence to produce a "flameless powder" as hereinbefore defined using M. D. cordite as a basis it is necessary to add approximately 16 parts of starch to 100 parts of the ingredients of which M. D. cordite is composed. Applying the same considerations to other powders in use we arrive at the following figures as representing the quantity of starch that should

be added to 100 parts of the propellant mixture in each case:

|                                                         |    |
|---------------------------------------------------------|----|
| 7 parts of starch per 100 parts American pyrocollodion. | 70 |
| 14 parts of starch per 100 part Norwegian ballistite.   |    |
| 28 parts of starch per 100 parts Mk. I. cordite.        |    |
| 33 parts of starch per 100 parts Italian ballistite.    | 75 |

From the above it follows that a greater quantity of starch or the like must be added in order to eliminate flame from high velocity guns of larger caliber, but that the specific pressure or power of the powder will be lowered by such an addition, so that it may be necessary to increase the size of the chamber of such large guns in order to take the increased charge; at the same time, however, the erosion is greatly reduced. Thus we arrive at the following figures:

| Powder.                                 | Pressure developed when fired at 0.23 in ton per square inch. | Calorimetric value at 10 tons water liquid per gram. | Erosion in grams of steel carried away in one shot. |    |
|-----------------------------------------|---------------------------------------------------------------|------------------------------------------------------|-----------------------------------------------------|----|
| M. D. cordite.....                      | 17.10                                                         | 1025                                                 | 100.0                                               | 90 |
| M. D. cordite + 40 parts of starch..... | 11.65                                                         | 660                                                  | 11.8                                                | 95 |

It must, however, be admitted that calculations of this nature are exceedingly complex, so that those less skilled in the art may be desirous of arriving at a close approximation by making use of the fact that for propellants of a similar nature the pyrometric value will be approximately proportionate to the calorimetric value; for the use of such the following table is appended whereby they can by the simple process of interpolation arrive at a very close approximation to the quantity of starch that should be added to any propellant mixture or basis of any given calorimetric value:

| Nature of propellant mixture used. | Calorimetric value of propellant mixture used (water liquid determined at 10 tons per square inch calories per gram). | Approximate number of parts of starch that should be added to 100 parts of propellant mixture in question in order to produce a "flameless powder" as hereinbefore defined. |     |
|------------------------------------|-----------------------------------------------------------------------------------------------------------------------|-----------------------------------------------------------------------------------------------------------------------------------------------------------------------------|-----|
| American pyrocollodion.....        | 800                                                                                                                   | 7.0                                                                                                                                                                         | 115 |
| Norwegian ballistite.....          | 995                                                                                                                   | 14.0                                                                                                                                                                        |     |
| Walsrode.....                      | 1020                                                                                                                  | 15.5                                                                                                                                                                        |     |
| M. D. cordite.....                 | 1025                                                                                                                  | 16.0                                                                                                                                                                        |     |
| Mk. I. cordite.....                | 1250                                                                                                                  | 28.0                                                                                                                                                                        | 120 |
| Sporting ballistite.....           | 1295                                                                                                                  | 30.0                                                                                                                                                                        |     |
| Italian ballistite.....            | 1325                                                                                                                  | 33.0                                                                                                                                                                        | 125 |

Throughout this specification and in particular in the claims at the conclusion thereof, I use the term nitrocellulose to include any variety of nitrocellulose, namely the variety insoluble in ether-alcohol commonly known as guncotton and also the soluble variety known as soluble cotton or pyrocollodion. In carrying my invention into effect it is merely necessary to incorporate the material which goes to make up the propellant basis in the presence of a gelatinizing agent and preferably that normally used for such mixtures as constitute the basis, for example acetone where guncotton or insoluble nitrocellulose is present and ether alcohol where soluble nitrocellulose or pyrocollodion is present, and to incorporate, preferably after gelatinization is complete, the necessary quantity of starch into the "dough" then to form the "dough" into the desired shape and size and dry the product in the usual manner. Thus, according to one example in which I use a mixture of nitrocellulose, nitroglycerin and vaseline as the basis I proceed as follows:

307 lbs. of nitrocellulose containing 13.3% nitrogen is mixed with 440 lbs. of nitroglycerin and the mixture rubbed through a sieve in the usual manner. This mixture of 30 nitrocellulose and nitroglycerin is then charged into an incorporator, preferably of the Werner Pfleiderer type, and 100 lbs. of acetone added and the mass incorporated for 6 hours; 39 lbs. of vaseline and 214 lbs. of 35 starch in a fine state of division are then added; the whole is then incorporated for a further period of 2 hours; during the period of incorporation 87½ lbs. of acetone is added as required, after which the dough is 40 pressed into cords or tubes of the desired size and dried in the usual manner. The propellant so obtained will be a "flameless powder" as hereinbefore defined, and less erosive than any known artillery powder 45 and far more powerful than any of the less erosive powders now in use, its properties in these respects being as set forth in the following table wherein the power and erosive properties of modern artillery powders are 50 also set forth for comparison, taking cordite M. D. as 100:

| 55 | Powder.                     | Erosive properties<br>in grains of steel<br>carried away per<br>shot. | developed<br>pressure when dried<br>at a density of<br>0.23 in tons per<br>square inch. |
|----|-----------------------------|-----------------------------------------------------------------------|-----------------------------------------------------------------------------------------|
| 60 | New flameless powder.....   | 46.6                                                                  | 15.65                                                                                   |
|    | French B. N.....            | 50.0                                                                  | 14.90                                                                                   |
|    | American pyrocollodion..... | 51.0                                                                  | 14.80                                                                                   |
|    | Norwegian ballistite.....   | 96.5                                                                  | 16.85                                                                                   |
|    | Cordite M. D.....           | 100.0                                                                 | 17.40                                                                                   |
|    | Cordite Mk. I.....          | 173.0                                                                 | 19.25                                                                                   |
|    | Italian Ballistite.....     | 218.0                                                                 | 18.45                                                                                   |

According to another example in which I 65 use soluble nitrocellulose as a basis and man-

ufacture a product containing 10% more starch than is necessary to produce a flameless powder I proceed as follows:

600 lbs. (dry weight) of moist soluble nitrocellulose is freed from water by displacing said water with alcohol in the usual manner, after which the excess of alcohol is removed by means of hydraulic pressure, also in the usual manner. The soluble nitrocellulose containing about 200 lbs. of alcohol is then transferred into a suitable incorporator and incorporated for about 6 hours during which time an amount of ether equal to about twice the weight of the alcohol originally left in the charge is added. 75 After this 114 lbs. of starch is added together with a further addition of solvent if required and incorporation continued for a further 2 hours. The dough so produced is then formed into the desired size and shape 80 and finally dried in the usual manner. The resulting product will be found to be flameless not only in the weapons above mentioned but also in guns and howitzers of somewhat larger caliber; it is, however, low 85 in power so that I prefer to use it admixed with an ordinary smokeless powder which without such admixture would produce a flame and to use a quantity of this new product equal to ten times the weight of 90 starch required as hereinbefore set forth, as for example—

(a) American pyrocollodion— 100  
New product ----- 70 100

or (b) Walsrode ----- 100  
New product ----- 155

Such mixtures will be found to be "flameless powders" as hereinbefore defined.

Having thus described my invention what I claim as such and desire to secure by Letters Patent is:

1. In the manufacture of propellant explosives, the addition of starch to the basic propellant, in such quantity as to reduce below their ignition point the temperature of the gases evolved upon the firing of the said propellant in suitable guns as hereinbefore set forth. 110

2. In the manufacture of propellant explosives, the addition of starch to the basic propellant, in quantity greater than is necessary to reduce below their ignition point the temperature of the gases evolved upon the firing of the said propellant, in suitable 120 guns as hereinbefore set forth.

3. In the manufacture of propellant explosives, the addition of starch to the basic propellant in such quantity as to reduce below their ignition point the temperature of 125 the gases evolved upon the firing of the said propellant, in suitable guns as hereinbefore set forth, said starch being incorporated with the material of said propellant in presence of a gelatinizing agent. 130

4. In the manufacture of propellant explosives, the addition to the basic propellant of an organic compound containing a preponderance of H—C—OH groups, in such quantity as to reduce below their ignition point the temperature of the gases evolved upon the firing of said propellant in suitable guns as hereinbefore set forth. 60
5. In the manufacture of propellant explosives, the addition to the basic propellant of an organic compound containing a preponderance of H—C—OH groups, said compound being incorporated with the material of said propellant in presence of a 65 gelatinizing agent, and in such quantity as to reduce below their ignition point the temperature of the gases evolved upon the firing of said propellant in suitable guns as hereinbefore set forth. 70
- 10 6. In the manufacture of propellant explosives, the addition to the basic propellant of organic compounds containing a preponderance of H—C—OH groups, in such quantity as to reduce below their ignition 75 point the temperature of the gases evolved upon the firing of the said propellant in suitable guns as hereinbefore set forth. 80
- 15 7. In the manufacture of propellant explosives, the addition to the basic propellant of organic compounds containing a preponderance of H—C—OH groups, said compounds being incorporated with the material of said propellant in presence of a gelatinizing agent, and in such quantity as 85 to reduce below their ignition point the temperature of the gases evolved upon the firing of the said propellant in suitable guns as hereinbefore set forth. 90
- 20 8. In the manufacture of propellant explosives, containing nitrocellulose, the addition of starch to said nitrocellulose in such quantity as to reduce below their ignition 95 point the temperature of the gases evolved upon the firing of the said propellant in suitable guns as hereinbefore set forth. 100
- 25 9. In the manufacture of propellant explosives, containing nitrocellulose, the addition of starch to such nitrocellulose in such quantity as to reduce below their ignition 105 point the temperature of the gases evolved upon the firing of the said propellant in suitable guns as hereinbefore set forth, said starch being incorporated with said nitrocellulose in presence of gelatinizing agent. 110
- 30 10. In the manufacture of propellant explosives containing nitrocellulose, the addition to said nitrocellulose of an organic compound containing a preponderance of H—C—OH groups, in such quantity as to 115 reduce below their ignition point the temperature of the gases evolved upon the firing of the said propellant in suitable guns as hereinbefore set forth. 120
- 35 11. In the manufacture of propellant explosives containing nitrocellulose, the addition to said nitrocellulose of an organic compound containing a preponderance of H—C—OH groups, said compound being incorporated with said nitrocellulose in presence of a gelatinizing agent and in such 125 quantity as to reduce below their ignition point the temperature of the gases evolved upon the firing of the said propellant in suitable guns as hereinbefore set forth. 130
- 40 12. In the manufacture of propellant explosives containing nitrocellulose, the addition to said nitrocellulose of organic compounds containing a preponderance of H—C—OH groups, in such quantity as to reduce below their ignition point the temperature of the gases evolved upon the firing of the said propellant in suitable guns as hereinbefore set forth. 135
- 45 13. In the manufacture of propellant explosives containing nitrocellulose, the addition to said nitrocellulose of organic compounds containing a preponderance of H—C—OH groups, said compounds being incorporated with said nitrocellulose in presence of a gelatinizing agent and in such 140 quantity as to reduce below their ignition point the temperature of the gases evolved upon the firing of the said propellant in suitable guns as hereinbefore set forth. 145
- 50 14. The manufacture of a "flameless powder" as hereinbefore defined by incorporating a compound with a preponderance of H—C—OH groups with nitrocellulose and with a gelatinizing agent substantially as hereinbefore described. 150
- 55 15. The manufacture of a "flameless powder" as hereinbefore defined by incorporating a compound containing a preponderance of H—C—OH groups with mixtures containing nitrocellulose and with a gelatinizing agent substantially as hereinbefore described. 155
- 60 16. A "flameless powder" as hereinbefore defined composed substantially of a mixture of nitrocellulose 30.7%, nitro-glycerin 44%, vaseline 3.9% and starch 21.4% as hereinbefore described. 160
- In testimony whereof I have affixed my signature in presence of two witnesses.
- OSWALD SILBERRAD.
- Witnesses:
- VICTOR F. FEENY,  
CYRIL J. FEENY.